

Patented Aug. 15, 1944

2,355,770

# UNITED STATES PATENT OFFICE

2,355,770

## PREPARATION OF CYCLO-TRIMETHYLENE-TRINITRAMINE

Joseph A. Wyler, Allentown, Pa., assignor to  
Trojan Powder Company, Allentown, Pa.

No Drawing. Application January 12, 1943,  
Serial No. 472,167

8 Claims. (Cl. 260—248)

This invention relates to the nitration of hexamethylenetetramine to cyclo-trimethylenetrinitramine commonly called "Hexogen" or "Cyclonite."

It is well known that hexamethylenetetramine can be nitrated to cyclo-trimethylenetrinitramine by means of concentrated nitric acid, particularly an acid of a strength greater than 92% HNO<sub>3</sub>. However, in all known processes, the yields are usually low—varying from 62% to 72% of theory.

It is also well known that the process of nitration which introduces either a nitrate group or a nitro group into an organic compound is usually improved by the presence of dehydrating agents in the nitrating bath. This improvement is generally in the yield of the nitrated product. Agents which are known to increase such yields are sulfuric acid, oleum, SO<sub>3</sub>, phosphoric acid, P<sub>2</sub>O<sub>5</sub>, etc.

In the nitration of hexamethylenetetramine to Hexogen, we are concerned with the formation of a nitramine, that is, the introduction of an NO<sub>2</sub> group into an amine to form a nitrogen to nitrogen and not a nitrogen to carbon bond. Also, we are concerned with the removal of a methylene amine substituent within the ring structure of the hexamethylenetetramine. Thus, hexamethylenetetramine:



upon nitration forms



with the methylene amine substituent:



being set free and altered. The changes undergone by this latter substituent are not thoroughly known. It is known

that most of the —CH<sub>2</sub>— groups form CH<sub>2</sub>O and the evidence indicates the formation of only a small amount of NH<sub>3</sub> under ideal nitrating conditions.

5 The presence of the CH<sub>2</sub>O in the nitrating bath is, however, a very important factor due to the ease of oxidation of CH<sub>2</sub>O by nitric acid, particularly by mixtures of nitric acid and dehydrating agents, and this oxidation has a very deleterious effect upon the yield of Hexogen obtained in the nitration.

Now, I have found that in the nitration of hexamethylenetetramine using nitric acid in combination with such powerful dehydration agents as mentioned above results are obtained which are no longer what would be expected on the basis of known facts regarding the use of these agents in well known nitrations. Thus, the addition of sulfuric acid or sulfuric acid and SO<sub>3</sub> to a HNO<sub>3</sub> used for the nitration of hexamethylenetetramine does not improve the yield of nitration but actually lowers it; whereas, phosphoric acid, hydrated P<sub>2</sub>O<sub>5</sub>, or phosphoric acid and P<sub>2</sub>O<sub>5</sub>, or P<sub>2</sub>O<sub>5</sub>, do increase the yield of nitration when used under certain restricted conditions which will be indicated below.

15 The principal object of my invention is to nitrate hexamethylenetetramine to Hexogen with a greater yield. Other objects will become apparent upon a further perusal of this specification.

20 In order more clearly to point out my invention, the following examples, in which all parts are by weight, are given.

25

### Example #1

30 8 parts of hexamethylenetetramine were added, over a period of 12 minutes, with stirring, to 100 parts of 99% nitric acid, to which 5 parts of 104.62% H<sub>2</sub>SO<sub>4</sub> had been added, keeping the temperature of the nitrating bath at 3° to 10° C. throughout the nitration. The mixture was stirred at about 5° C. for 15 minutes after all the hexamethylenetetramine had been added, when 35 it was drowned in a large excess of cold water and the precipitated cyclo-trimethylenetrinitramine filtered off, washed with cold water, then with hot water, with alcohol and finally dried at 60° C. to constant weight. The yield of cyclo-40 trimethylenetrinitramine obtained was 9 parts or 71% of theory. Using the same nitric acid, without the addition of any sulfuric acid, the yield was 72% of theory indicating that the addition of this small amount of 104.62% oleum did not improve the yield of Hexogen obtained.

*Example #2*

Using 12 parts of hexamethylenetetramine in place of the 8 parts in Example #1 and proceeding in the same manner a yield of Hexogen of 12 parts or 63% of theory was obtained, indicating a poor yield.

*Example #3*

Repeating Example #1, but using 15 parts of 104.62% sulfuric acid instead of 5 parts, gave a yield of Hexogen of 8 parts or only 63% of theory.

*Example #4*

Repeating Example #1, but using 20 parts of 104.62% sulfuric acid instead of 5 parts, gave a yield of Hexogen of 8 parts, or 63% of theory.

These examples are given to show that the presence of sulfuric acid or sulfuric acid and  $\text{SO}_3$  in the nitric acid does not improve its nitrating qualities, when used on hexamethylenetetramine, but actually lowers it, particularly as the concentration of  $\text{H}_2\text{SO}_4$  is increased.

*Example #5*

7 parts of hexamethylenetetramine were added, over a period of 12 minutes, with stirring, to 100 parts of 99% nitric acid to which 3 parts of  $\text{P}_2\text{O}_5$  had been added. The temperature of the nitrating bath was held at 0° to 5° C. throughout the nitration. The mixture was stirred at about 5° C. for 15 minutes after all the hexamethylenetetramine had been added, when it was drowned in a large excess of cold water and the thus precipitated cyclo-trimethylenetrinitramine filtered off, washed with cold water, then with hot water, then with alcohol and finally dried at 60° C. to constant weight. The yield of Hexogen obtained was 9 parts or 81% of theory.

*Example #6*

Example #5 was repeated, using 6 parts of  $\text{P}_2\text{O}_5$  instead of 3 parts. The yield obtained was 10 parts or 90% of theory.

*Example #7*

Example #5 was repeated, using 10 parts of  $\text{P}_2\text{O}_5$  instead of 3 parts. The yield obtained was 10 parts, or 90% of theory.

*Example #8*

Using 20 parts of  $\text{P}_2\text{O}_5$  and 8 parts of hexamethylenetetramine and proceeding as above gave a yield of 11 parts, or 87% of theory.

*Example #9*

Repeating Example #8, but using 10 parts of Hexamethylenetetramine gave a yield of 82% of theory.

*Example #10*

4 parts of hexamethylene tetramine were added, over a period of 10 minutes, with stirring, to 100 parts of 99% nitric acid, to which 10 parts of  $\text{P}_2\text{O}_5$  had been added. After the addition of the hexamethylenetetramine, 4 parts of  $\text{P}_2\text{O}_5$ , followed by 4 parts of hexamethylenetetramine and after the addition of the latter, 7 parts of  $\text{P}_2\text{O}_5$  followed by 4 parts of hexamethylenetetramine were added. The temperature was held between 0° C. and 12° C. and the nitration mixture stirred for 15 minutes after the last addition of hexamethylenetetramine. The nitration mixture was poured into a large volume of cold water and handled in the same manner as under Example #1. The yield of Hexogen obtained was 17 parts

from 12 parts of hexamethylenetetramine or 90% of theory.

*Example #11*

Repeating experiment #10, with the additional steps of adding 4 additional parts of  $\text{P}_2\text{O}_5$  and 4 additional parts of hexamethylenetetramine the yield of Hexogen obtained was 19 parts from 16 parts of hexamethylenetetramine or 75% of theory. It should be noted that in this experiment 16 parts of hexamethylenetetramine and 25 parts of  $\text{P}_2\text{O}_5$  were used for 100 parts of 99%  $\text{HNO}_3$ .

My work has shown that the use of more than about 25 parts of  $\text{P}_2\text{O}_5$  for each 100 parts of nitric acid, calculated to 100% strength, is no longer effective in improving the yield of Hexogen in the nitration. Consequently, my invention is limited to the use of not more than about 25 parts of  $\text{P}_2\text{O}_5$  to 100 parts of nitric acid (100%).

Also, my best results are obtained by regulating the  $\text{P}_2\text{O}_5$  or water content of the nitrating acid to within certain limits during the nitration, that is, my best results are obtained when the nitrating acid is close to anhydrous  $\text{HNO}_3$  throughout the nitration. It should be noted that although my best yields are obtained under anhydrous conditions I also obtain important improvements in yield with nitric acids of lower strengths, that is, as low as about 85-90%  $\text{HNO}_3$ . Consequently, my process is applicable to the use of nitric acid of a strength greater than about 85-90%  $\text{HNO}_3$  treated with any amount of  $\text{P}_2\text{O}_5$  not greater than about 25 parts of  $\text{P}_2\text{O}_5$  per 100 parts of nitric acid (100%).

In this specification the term "concentrated nitric acid" is used to cover any strength greater than about 85 to 90%  $\text{HNO}_3$ .

My work has shown that a nitrating acid comprising  $\text{HNO}_3$  and  $\text{H}_3\text{PO}_4$ ; or  $\text{HNO}_3$ ,  $\text{H}_3\text{PO}_4$  and  $\text{P}_2\text{O}_5$ ; or  $\text{HNO}_3$  and  $\text{P}_2\text{O}_5$  in such proportions that the free water content of the nitrating acid is not greater than about 4% and the negative water content not greater than about 4%, is the most practicable nitrating acid from the standpoint of yield of Hexogen from a given amount of hexamethylenetetramine.

The term "negative water content," as appearing in the specification and the claims, is used to designate the analytical result obtained on a given nitrating acid by adding the "% nitric acid," the total phosphate calculated to "%  $\text{H}_3\text{PO}_4$ " and the "%  $\text{NO}_2$ " in the acid and taking the difference between this sum and 100% as the water content; if the sum is greater than 100%, it shows that "negative water" is present and the difference between this sum and 100% gives the "% negative water."

I wish to emphasize that the examples and theories given above are merely illustrative or explanatory in nature and are not intended to limit my invention in any way not indicated by the appended claims. Thus I may use any temperature below about 30° C., although I prefer a range of from about 5° C. to 20° C.; I may use any ratio of hexamethylenetetramine to  $\text{HNO}_3$  up to about 16 parts of hexamethylenetetramine to 100 parts of 100%  $\text{HNO}_3$ ; I may add the hexamethylenetetramine and the  $\text{P}_2\text{O}_5$  simultaneously or successively; I may vary the rates of addition of reactants and times of stirring over a wide range or I may alter the method of recovery of the Cyclonite from the nitrating bath without departing from the essence of my invention. Also, in all my examples, I have mentioned  $\text{P}_2\text{O}_5$

as the dehydrating agent added, but since  $P_2O_5$  in contact with water forms  $H_3PO_4$  and other hydrates it is understood that I may at times use  $H_3PO_4$ , or  $P_2O_5$  in other states of hydration instead of  $P_2O_5$  itself. Consequently, my use of the term  $P_2O_5$  in the description may at times cover the " $P_2O_5$  equivalent" of the hydrated  $P_2O_5$  present in the nitrating bath and is not intended to convey the thought that the  $P_2O_5$  necessarily exists in the solution as anhydrous  $P_2O_5$ . It is understood that  $P_2O_5$  cannot exist in the anhydrous condition in contact with water.

I claim:

1. The process for the nitration of hexamethylenetetramine to cyclo-trimethylenetrinitramine which comprises reacting hexamethylenetetramine, at a nitrating temperature, with concentrated nitric acid containing a phosphorus pentoxide, said phosphorus pentoxide being present in an amount not in excess of 25 parts, by weight, of  $P_2O_5$  per 100 parts, by weight of nitric acid (100%), and said hexamethylenetetramine being added in an amount not in excess of 16 parts, by weight, of hexamethylenetetramine per 100 parts, by weight, of 100%  $HNO_3$ ; adding the reaction mixture to an excess of cold water, with stirring, and filtering off the cyclo-trimethylenetrinitramine which precipitates.

2. The process for the nitration of hexamethylenetetramine to cyclo-trimethylenetrinitramine which comprises reacting hexamethylenetetramine, at a nitrating temperature, with concentrated nitric acid containing a hydrated phosphorus pentoxide, said hydrated phosphorus pentoxide being present in an amount not in excess of 25 parts, by weight, of  $P_2O_5$  per 100 parts, by weight, of nitric acid (100%) and said hexamethylenetetramine being added in an amount not in excess of 16 parts, by weight, of hexamethylenetetramine per 100 parts, by weight, of 100%  $HNO_3$ ; adding the reaction mixture to an excess of cold water, with stirring, and filtering off the cyclo-trimethylenetrinitramine which precipitates.

3. The process for the nitration of hexamethylenetetramine to cyclo-trimethylenetrinitramine which comprises reacting hexamethylenetetramine, at a nitrating temperature, with concentrated nitric acid containing  $P_2O_5$ , said  $P_2O_5$  being present in an amount not in excess of 25 parts, by weight, of  $P_2O_5$  per 100 parts, by weight, of nitric acid (100%), and said hexamethylenetetramine being added in an amount not in excess of 16 parts, by weight, of hexamethylenetetramine per 100 parts, by weight, of 100%  $HNO_3$ ; adding the reaction mixture to an excess of cold water, with stirring, and filtering off the cyclo-trimethylenetrinitramine which precipitates.

4. The process for the nitration of hexamethylenetetramine to cyclo-trimethylenetrinitramine which comprises adding hexamethylenetetramine, with stirring, at a temperature below 30° C., to a concentrated nitric acid containing a phosphorus pentoxide; said hexamethylenetetramine being added in an amount not in excess of 16 parts, by weight, of hexamethylenetetramine per 100 parts, by weight, of 100%  $HNO_3$ ; said phos-

phorus pentoxide being present in an amount not in excess of 25 parts, by weight, of  $P_2O_5$  per 100 parts, by weight, of nitric acid (100%); adding the nitration mixture, with stirring, to an excess of cold water and filtering off the cyclo-trimethylenetrinitramine which precipitates.

5. The process for the nitration of hexamethylenetetramine to cyclo-trimethylenetrinitramine which comprises adding hexamethylenetetramine, 10 with stirring, at a temperature below 30° C., to a concentrated nitric acid containing a hydrated phosphorus pentoxide; said hexamethylenetetramine being added in an amount not in excess of 16 parts, by weight, of hexamethylenetetramine 15 per 100 parts, by weight, of 100%  $HNO_3$ ; said hydrated phosphorus pentoxide being present in an amount not in excess of 25 parts, by weight, of  $P_2O_5$  per 100 parts, by weight, of nitric acid (100%); adding the nitration mixture, with stirring, to an excess of cold water and filtering off the cyclo-trimethylenetrinitramine which precipitates.

6. The process for the nitration of hexamethylenetetramine to cyclo-trimethylenetrinitramine 20 which comprises adding hexamethylenetetramine, with stirring, at a temperature below 30° C., to a concentrated nitric acid containing  $P_2O_5$ ; said hexamethylenetetramine being added in an amount not in excess of 16 parts, by weight, of hexamethylenetetramine per 100 parts, by weight, of 100%  $HNO_3$ ; said  $P_2O_5$  being present in an amount not in excess of 25 parts, by weight, of  $P_2O_5$  per 100 parts, by weight, of nitric acid (100%); adding the nitration mixture, with stirring, to an excess of cold water and filtering off the cyclo-trimethylenetrinitramine which precipitates.

7. The process for the nitration of hexamethylenetetramine to cyclo-trimethylenetrinitramine 25 which comprises adding hexamethylenetetramine, with stirring, at a temperature below 30° C., to a concentrated nitric acid containing phosphoric acid; said hexamethylenetetramine being added in an amount not in excess of 16 parts, by weight, of hexamethylenetetramine per 100 parts, by weight, of 100%  $HNO_3$ ; said phosphoric acid being present in an amount not in excess of 25 parts, by weight, of  $P_2O_5$  per 100 parts, by weight, of nitric acid (100%); adding the nitration mixture, with stirring, to an excess of cold water and filtering off the cyclo-trimethylenetrinitramine which precipitates.

8. The process for the nitration of hexamethylenetetramine to cyclo-trimethylenetrinitramine 30 which comprises adding hexamethylenetetramine, with stirring, at a temperature below 30° C., to a nitric acid containing between 4% of free water and 4% of "negative water"; said water-range being produced by the addition of  $P_2O_5$  to the nitric acid; and said  $P_2O_5$  being added in an amount not in excess of 25 parts, by weight, of  $P_2O_5$  per 100 parts, by weight, of  $HNO_3$  (100%); adding the reaction mixture, with stirring, to an excess of cold water, filtering off the cyclo-trimethylenetrinitramine which precipitates, washing with water and drying.

JOSEPH A. WYLER.